

Jan. 29, 1957

R. I. JAFFEE ET AL

2,779,677

TI-SN-AL ALLOYS WITH ALPHA, BETA AND COMPOUND FORMERS

Filed Dec. 28, 1953

COMPARATIVE STRENGTHENING  
EFFECTS OF Al, Sb AND Sn ALLOY  
ADDITIONS TO COMMERCIAL  
PURITY Ti-BASE



INVENTORS.  
ROBERT I. JAFFEE,  
HORACE R. OGDEN,  
BY DANIEL J. MAYKUTH.

*Ward Crosby & Neal*  
ATTORNEYS.

# United States Patent Office

2,779,677

Patented Jan. 29, 1957

1  
2,779,677

## Ti-Sn-Al ALLOYS WITH ALPHA, BETA AND COMPOUND FORMERS

Robert I. Jaffee, Worthington, and Horace R. Ogden and Daniel J. Maykuth, Columbus, Ohio, assignors, by mesne assignments, to Rem-Cru Titanium, Inc., Midland, Pa., a corporation of Pennsylvania

Application December 28, 1953, Serial No. 400,744

14 Claims. (Cl. 75—175.5)

This invention pertains to improvements in titanium base alloys, and provides a series of alloys of high strength and ductility, and, as to certain analyses, also of high contamination resistance and high strength at elevated temperatures, and containing as essential constituents titanium, tin and aluminum, together with one or more additional metals selected from the groups comprising alpha promoters, beta promoters and compound formers as enumerated below.

This application is a continuation-in-part of applicants' prior applications Serial Nos. 151,314, filed March 22, 1950, now abandoned; 209,905, filed February 7, 1951, now abandoned; 253,564, filed October 27, 1951, now abandoned; 213,681 to 213,687, inc., all filed March 2, 1951, now abandoned; 285,076, filed April 29, 1952, now Patent No. 2,669,513, granted Feb. 16, 1954; and 294,263, filed June 18, 1952, now abandoned.

The aluminum content may be present over a broad range of about 0.25 to 8% and preferably about 1 to 8%.

The tin content may be present over a broad range of about 1 to 23%, with a preferred lower limit of about 2.5%, as adjudged from the standpoint of good room temperature mechanical properties, and a preferred lower limit of about 5% as regards the imparting of high contamination resistance at elevated temperatures. To the titanium-tin-aluminum alloy aforesaid, there may advantageously be added up to about 20% in aggregate of one or more of the other alpha promoters, up to about 50% in aggregate of one or more of certain of the beta promoters, and up to about 2 or 3% in aggregate of the compound formers, all as set forth more in detail hereinafter. For further enhancing the mechanical properties, the alloys of the invention may contain controlled amounts of the interstitials, carbon, oxygen and nitrogen. For certain analyses, as set forth below, carbon may be present up to about 1%, oxygen up to about 0.5% and nitrogen up to about 0.4%. When the total tin and aluminum content is below about 5%, and particularly when below about 2.5%, substantial additions of one or more of the interstitials carbon, oxygen and nitrogen or of metal of the alpha and/or beta promoter groups, is required for imparting high tensile properties for commercial applications, as elaborated upon below.

As above stated, the alloys of the invention are in general characterized by excellent room temperature mechanical properties, possessing high tensile strength as compared to the unalloyed titanium base metal or as compared to the corresponding binary titanium-tin and titanium-aluminum alloys, combined with adequate ductility for both hot and cold forming operations, i. e., forging, rolling, drawing, extruding, etc. For tin contents up to about 16%, they may likewise, in general, be welded without appreciable loss of ductility in the welded as compared to the non-welded portions. This is particularly true as regards those alloys having an all-alpha microstructure, and also as to certain of those having a beta-

2

containing microstructure, as explained more in detail below.

For imparting a high degree of contamination resistance, i. e., resistance against penetration by atmospheric gases, particularly oxygen and nitrogen, at elevated temperatures up to about 1100° C., the alloys should contain upwards of about 5% tin, although lesser amounts down to about 2% tin, are materially beneficial in this respect. Tin alloyed with titanium base metal appears to be unique in imparting this contamination resistance, and its effect is quite critical with respect to the degree of contamination resistance imparted commencing at a minimum of about 5% tin.

These contamination resistant alloys are also characterized by free scaling properties resulting from exposure to elevated temperatures up to about 1100° C. and to atmospheric, oxidizing, or alternately oxidizing and reducing conditions. That is to say, the scale formed is easily brushed off or flakes off during hot forming operations, such as forging or rolling.

Test results in support of the above are given in a cPending joint application of the present applicants Jaffee and Ogden and W. L. Finlay, Serial No. 341,796, filed March 11, 1953, now Patent No. 2,669,514.

As is known, the metal titanium in the pure state, is capable of existing in either of two allotropic forms. Below a temperature of about 885° C. or 1625° F., it assumes a close-packed hexagonal structure known as the alpha phase, while at this temperature and above, it assumes a body-centered cubic structure known as the beta phase.

Certain substitutional alloying additions to the titanium base metal, among which may be mentioned aluminum, tin, antimony, indium, silver, bismuth, lead, cadmium, zinc, and thallium as well as the interstitials carbon, oxygen and nitrogen may be termed alpha stabilizers or alpha promoters. The term alpha stabilizer includes those elements which raise the transformation range sharply, such as aluminum, oxygen, and nitrogen. Also alpha stabilizers include elements such as carbon, which have a relatively small solubility in alpha titanium, but which raise the transformation temperature for that amount which is in solution. Alpha stabilizers also include those elements such as tin, antimony, indium, and silver which have relatively large solubilities, of about the same magnitude, in both the alpha and beta phases and which have little effect on the transformation temperature range, neither raising nor lowering it markedly. A common characteristic of all alpha stabilizers, as we are considering them here, is that little or no hardening occurs in the thermal processing. The resulting alloys are, at room temperature, always all alpha in structure regardless of the heat treatment, including quenching or aging. Actually little is known concerning the specific effects of bismuth, lead, cadmium, zinc, and thallium on the transformation range. These alloying elements produce alloys which fit the criteria given, namely, that they form all-alpha alloys, which do not retain any substantial content of beta phase nor harden appreciably on quenching from the beta field. Hence these elements appear properly classified as alpha promoters, and will be so treated in this application.

Other substitutional alloying elements, when added in progressively increasing quantities, stabilize the beta phase at progressively lower temperatures, until a mixed alpha-beta or stable all-beta microstructure is obtained at normal or atmospheric temperatures, or the beta phase undergoes a eutectoid reaction, depending on the character and amount of the beta stabilizers added as discussed below.

Speaking in broadest terms, the beta stabilizers are Mo, V, Cr, Ta, Zr, Mn, Cr, Fe, W, Ni, Co and Cu. Silicon and beryllium may also be considered as beta stabilizing elements, but their solubilities in titanium are

relatively so slight and the tendency of the beta phase stabilized by these elements to decompose into eutectoid products so great, that it is equally proper to consider them as compound-forming elements. Within this broad category, however, only certain of the elements mentioned are suitable for producing mixed-phase, alpha-beta alloys, or all-beta alloys. These are the elements which have beta-isomorphous diagrams, or which have beta-eutectoid diagrams such that the decomposition of the beta phase into eutectoid is so sluggish that the alloys behave like those in a beta-isomorphous system. The beta stabilizing elements of this type are Mo, V, Cb, Ta, Mn, Fe and Cr. Tungsten is a borderline element as between the sluggishly decomposing and rapidly decomposing types and hence may be classified either way. Within this limited group only Mo, V, Cb and Ta are beta-isomorphous. They form the most thermally stable beta-containing alloys, as a result of their beta-isomorphism.

Zirconium is a beta promoter or stabilizer in the sense that the lowest temperature at which alloys thereof with titanium are entirely beta, becomes progressively lower with increasing amounts of zirconium, until a composition is reached at which this so-called beta transus temperature starts to increase again with further additions of zirconium. While zirconium thus lowers the transformation temperature of titanium, the alloys eventually revert to the alpha phase at lower temperatures unless other beta promoters are present. Zirconium is isomorphous with titanium both in the alpha and beta fields. As a result, it is proper to consider zirconium together with vanadium, molybdenum, columbium and tantalum as all being beta-isomorphous with titanium.

The use of copper alone as an alloying addition to titanium, does not fit into the above-mentioned grouping of beta-isomorphous and sluggishly decomposing eutectoid beta promoters, because the beta phase stabilized by copper always decomposes rather rapidly into pro-eutectoid and eutectoid products, and the same is generally true with respect to cobalt, nickel silicon and beryllium, above listed under the broad category of beta stabilizers. Copper, however, is a useful addition when present as a minor alloying element, for example, up to a few percent, in alloys containing larger amounts of other beta-stabilizing elements, within the narrow group of elements last mentioned above since, in these low concentrations and in the presence of such other beta-stabilizing elements, the tendency of the beta phase stabilized in part by copper to decompose into eutectoid products is minimized or entirely eliminated.

The tolerance of the ductile Ti-Sn-Al base alloys of the invention with respect to additions of the various beta promoters above mentioned, varies considerably for the individual elements of this group, being greatest with respect to those which form beta-isomorphous systems with titanium, and least for those which decompose most readily into eutectoid decomposition products. Thus, the Ti-Sn-Al base alloys may be strengthened without undue embrittlement by additions of up to about 50% in aggregate of elements composing the beta-isomorphous group, viz., molybdenum, vanadium, columbium, tantalum and zirconium, since these elements are soluble in all proportions in beta titanium. Of the sluggishly decomposing elements, the base alloy will tolerate additions of up to about 20% of either or both chromium and tungsten, up to about 10% manganese, and up to about 7% iron. Metal of the group cobalt, nickel and copper may be added up to a total of about 5%. For additions of all of the above-mentioned beta promoters, the lower effective limit is about 0.5% and preferably about 1%.

The tolerance of the ductile Ti-Sn-Al base alloys for the other alpha promoters depends on the amount of tin and aluminum present, the less tin and aluminum present, the greater the amount of other alpha promoters that can be added, and vice versa. Antimony may be added

to a maximum content of 18%. The preferred proportioning of the antimony content in relation to the tin and aluminum contents are given below. Indium may be added up to a maximum content of 15%. Silver may be added up to about 20%. Cadmium, zinc, thallium, bismuth and lead may be added up to 15% each, added to the charge in melting. The lower effective limit for the alpha promoters is about 0.5% and preferably about 1%.

The elements Ce, B, As, S, Te and P are strictly compound forming elements. They do not have appreciable solubilities in either the alpha or beta phases, but form intermetallic compounds with titanium. The beta promoters silicon and beryllium are likewise best grouped as compound forming elements, in view of their above-mentioned low solubilities in titanium and the tendency of the beta phase stabilized by these elements to decompose rapidly into eutectoid products. The Ti-Sn-Al base alloys of the invention will tolerate only relatively small amounts of these compound forming elements, i. e., up to a total of about 2 or 3% maximum, the lower effective limit being about 0.1 or 0.2%.

Substantially pure and ductile metallic titanium may be produced at considerable expense by the so-called "iodide" process described in U. S. Patent 1,671,213 to Van Arkel; while ductile titanium of commercial purity is produced more cheaply by the magnesium reduction of titanium tetrachloride by the process described in U. S. Patent 2,205,854 to Kroll. Both procedures, particularly the latter, result in some contamination of the titanium metal with one or more of the interstitials, carbon, oxygen and nitrogen. But since, as noted above, these are all alpha promoting or stabilizing elements, the resultant somewhat contaminated titanium metal obtained, has at room temperatures a single phase, all-alpha microstructure.

The all-alpha, all-beta and mixed alpha-beta alloys of titanium have their respective advantages and disadvantages. Generally speaking, the alpha alloys provide good all-around performance, having good weldability, and being strong and resistant to oxidation, both cold and hot, but are somewhat inferior as to ductility. The all-beta alloys, on the other hand, have excellent bendability and ductility, are strong both hot and cold, but are somewhat vulnerable to atmospheric contamination, particularly at elevated temperatures. The mixed alpha-beta alloys provide a compromise performance as between all-alpha and all-beta alloys, being strong when cold and warm, but weak hot, while possessing good bendability and ductility, with a moderate degree of resistance to atmospheric contamination.

Since the Ti-Sn-Al base alloys have, as above noted, an all-alpha microstructure, they may be readily welded in tin contents up to about 16%, with no appreciable impairment of ductility in the welded as compared to the non-welded portions. They also form an excellent base alloy for the quaternary and higher component alloys of the invention, that may be also welded without appreciable loss of ductility in the welded as compared to the non-welded portions. This is particularly true as regards the above-mentioned alpha-promoter additions to the base alloy. Also, in general, the quaternary and higher component alloys made by additions of the beta-isomorphous elements above designated, are weldable without appreciable impairment of ductility. It may furthermore be stated that in general the alpha-beta alloys according to the invention can be produced to have ductile welded portions if suitable post-welding heat treatments are applied as described in the co-pending application of Robert I. Jaffee, Horace R. Ogden and Ralph A. Happe, Serial No. 305,504, filed August 20, 1952 bearing common ownership.

In the ductile Ti-Sn-Al base alloys of the invention, the following Table A shows the preferred maximum aluminum content for any given tin content throughout the range above specified for these elements:

5  
TABLE A

| Percent Tin | Percent Aluminum Max. |
|-------------|-----------------------|
| 0.25        | 8                     |
| 1           | 6                     |
| 5           | 5                     |
| 10          | 4.5                   |
| 15          | 4                     |
| 20          | 3                     |
| 25          | 1                     |

Thus, for best results, as the tin content increases, the aluminum content should be decreased in the above proportions and vice versa.

Antimony is a particularly valuable addition to the Ti-Sn-Al base alloys of the invention, as it imparts thereto about the same strengthening effect as equivalent additions of tin or aluminum. This is shown by the following Table I presenting test data on room temperature mechanical properties which establish the upper limits for various combinations of antimony, tin and aluminum in titanium base alloys:

Table I.—Mechanical properties of Ti-Sb-Sn and Ti-Sb-Sn-Al alloys

(COMMERCIAL PURITY TI-BASE)

[These alloys were 980° C. forged, 850° C. rolled and annealed two hours at 850° C.]

| Composition, Percent<br>(Balance Titanium) | Tensile Properties: p. s. 1.1X1,000 |                      |                                |                                    | Vickers<br>Hardness | MBR, T |         |
|--------------------------------------------|-------------------------------------|----------------------|--------------------------------|------------------------------------|---------------------|--------|---------|
|                                            | 0.2<br>Percent<br>Offset<br>Yield   | Ultimate<br>Strength | Percent<br>Elongation<br>in 1" | Percent<br>Reduction<br>in<br>Area |                     | L      | T       |
| 6Sb                                        | 58                                  | 77                   | 22                             | 47                                 | 227                 | 1.5    | 1.6     |
| 5Sb-5Sn                                    | 74                                  | 94                   | 17                             | 46                                 | 262                 | 1.5    | 4.7     |
| 5Sb-10Sn                                   | 100                                 | 111                  | 17                             | 44                                 | 317                 | 2.5    | 3.2     |
| 5Sb-15Sn                                   | 129                                 | 131                  | 15                             | 46                                 | 330                 | 2.0    | 3.7     |
| 5Sb-17.5Sn                                 | 134                                 | 0                    | 6                              | 338                                |                     | 5.2    |         |
| 5Sb-20Sn                                   | (1)                                 | (1)                  | (1)                            | (1)                                | (1)                 | (1)    | (1)     |
| 10Sb                                       | 77                                  | 91                   | 19                             | 46                                 | 287                 | 2.5    | 2.5     |
| 10Sb-5Sn                                   | 100                                 | 111                  | 17                             | 44                                 | 317                 | 2.5    | 3.2     |
| 10Sb-10Sn                                  | 125                                 | 133                  | 16                             | 38                                 | 320                 | 4.9    | 4.9     |
| 10Sb-12.5Sn                                |                                     | 108                  | 0                              | 0                                  | 330                 | Br     | 7.0     |
| 10Sb-15Sn                                  | (1)                                 | (1)                  | (1)                            | (1)                                | (1)                 | (1)    | (1)     |
| 10Sb-17.5Sn                                | (1)                                 | (1)                  | (1)                            | (1)                                | (1)                 | (1)    | (1)     |
| 16Sb                                       | 99                                  | 111                  | 15                             | 43                                 | 304                 | 2.5    | 3.3     |
| 16Sb-5Sn                                   | 126                                 | 0                    | 6                              | 354                                | Br                  | Br     | Br      |
| 16Sb-7.5Sn                                 | (1)                                 | (1)                  | (1)                            | (1)                                | (1)                 | (1)    | (1)     |
| 10Sb                                       | 77                                  | 91                   | 19                             | 46                                 | 267                 | 1.5    | 1.6     |
| 7.5Sb-2.5Sn                                | 76                                  | 96                   | 16                             | 46                                 | 268                 | 2.3    | 3.1     |
| 5Sb-5Sn                                    | 74                                  | 94                   | 17                             | 46                                 | 262                 | 1.5    | 4.7     |
| 2.5Sb-7.5Sn                                | 81                                  | 98                   | 18                             | 43                                 | 270                 | 2.2    | 3.2     |
| 10Sn                                       | 77                                  | 92                   | 20                             | 46                                 | 278                 | 1.7    | 2.1     |
| 15Sb                                       | 99                                  | 111                  | 15                             | 43                                 | 304                 | 2.5    | 2.5     |
| 12.5Sb-2.5Sn                               | 109                                 | 117                  | 14                             | 42                                 | 311                 | 1.9    | 3.7     |
| 10Sb-5Sn                                   | 100                                 | 111                  | 17                             | 44                                 | 317                 | 2.5    | 3.2     |
| 5Sb-10Sn                                   | 107                                 | 116                  | 17                             | 39                                 | 325                 | 1.7    | 3.5     |
| 2.5Sb-12.5Sn                               | 109                                 | 118                  | 14                             | 36                                 | 313                 | 2.9    | 5.5     |
| 15Sn                                       | 107                                 | 117                  | 16                             | 45                                 | 348                 | 1.8    | 2.7     |
| 10Sb-2.5Al                                 | 123                                 | 125                  | 13                             | 38                                 | 351                 | 2.4    | 3.3     |
| 7.5Sb-2.5Sn-2.5Al                          | 110                                 | 115                  | 15                             | 48                                 | 339                 | 2.6    | 3.4     |
| 5Sb-5Sn-2.5Al                              | 114                                 | 118                  | 13                             | 44                                 | 343                 | 2.8    | 3.6/5.2 |
| 2.5Sb-7.5Sn-2.5Al                          | 110                                 | 117                  | 15                             | 40                                 | 345                 | 2.6    | 2.5     |
| 10Sn-2.5Al                                 | 113                                 | 119                  | 20                             | 43                                 | 345                 | 2.5    | 3.2     |
| 10Sb-2.5Al-0.2C                            | 143                                 | 146                  | 16                             | 47                                 | 393                 | 2.0    | 2.8/Br  |
| 7.5Sb-2.5Sn-2.5Al-0.2C                     | 136                                 | 137                  | 8                              | 24                                 | 402                 | 2.8    | 2.7/5.3 |
| 5Sb-5Sn-2.5Al-0.2C                         | 154                                 | 157                  | 5                              | 18                                 | 400                 | 6.2    | Br      |
| 2.5Sb-7.5Sn-2.5Al-0.2C                     | 144                                 | 146                  | 5                              | 21                                 | 390                 | 3.0    | 5.2     |
| 10Sn-2.5Al-0.2C                            | 140                                 | 141                  | 6                              | 29                                 | 395                 | 5.5    | Br      |
| 5Al-2.5Sb                                  | 110                                 | 117                  | 15                             | 42                                 | 352                 | 2.8    | 2.7/5.3 |
| 5Al-2Sb-0.5Sn                              | 103                                 | 109                  | 15                             | 43                                 | 351                 | 2.8    | 3.7     |
| 5Al-1.5Sb-1Sn                              | 106                                 | 113                  | 15                             | 37                                 | 346                 | 2.1    | 8.6     |
| 5Al-1Sb-1.5Sn                              | 103                                 | 112                  | 17                             | 46                                 | 343                 | 2.9    | 7.6     |
| 5Al-0.5Sb-2Sn                              | 100                                 | 111                  | 14                             | 43                                 | 348                 | 2.8    | 2.7     |
| 5Al-2.5Sn                                  | 101                                 | 110                  | 17                             | 47                                 | 344                 | 2.9    | 2.7     |
| 5Al-2.5Sb-0.2C                             | 128                                 | 134                  | 7                              | 21                                 | 389                 | 2.8    | 7.6     |
| 5Al-2Sb-0.5Sn-0.2C                         | (1)                                 | (1)                  | (1)                            | (1)                                | (1)                 | (1)    | (1)     |
| 5Al-1.5Sb-1Sn-0.2C                         | 132                                 | 135                  | 17                             | 42                                 | 394                 | 2.8    | 3.5     |
| 5Al-1Sb-1.5Sn-0.2C                         | 131                                 | 135                  | 17                             | 48                                 | 396                 | 2.8    | 2.8/5.5 |
| 5Al-0.5Sb-2Sn-0.2C                         | 130                                 | 134                  | 7                              | 28                                 | 391                 | 2.8    | 2.8/5.5 |
| 5Al-2.5Sn-0.2C                             | 134                                 | 135                  | 9                              | 25                                 | 400                 | 2.8    | 6.8     |

<sup>1</sup> Could not be fabricated.

The data of the above Table I establishes that antimony and tin are equivalent in strengthening effect when

For alloys of the invention containing tin approximating its lower limit, the following Table C shows the

substituted one or the other on a weight percentage basis, i. e., percent for percent. This data also establishes that 1% aluminum is roughly equivalent to 3% of tin or antimony in strengthening effect.

This equivalency is also shown by the accompanying drawing giving the 0.2% offset yield strengths for the Ti-Al, Ti-Sn and Ti-Sb binary alloys for varying percentages of the alloying additions.

For additions of antimony to the Ti-Sn-Al alloys of the invention, the following Table B shows the preferred maximum antimony content for given aluminum and tin contents:

TABLE B

| Percent Aluminum | Percent Tin | Percent Antimony Max. |
|------------------|-------------|-----------------------|
| 0.25             | 5           | 13                    |
| 1                | 5           | 11                    |
| 2                | 5           | 9                     |
| 3                | 5           | 7.5                   |
| 4                | 5           | 6                     |
| 5                | 5           | 5                     |

maximum permissible antimony content for any given aluminum content:

TABLE C

5

| Percent Alum-<br>num | Percent Antimony<br>Max. |
|----------------------|--------------------------|
| 0.25                 | 18.0                     |
| 1.0                  | 16.0                     |
| 2.0                  | 14.0                     |
| 3.0                  | 12.5                     |
| 4.0                  | 11.0                     |
| 5.0                  | 10.0                     |

Conversely, if the aluminum content approximates its lower limit, the following Table D shows the maximum permissible antimony content for any given tin content:

TABLE D

8

10

| Percent Tin | Percent Antimony Max. |
|-------------|-----------------------|
| 0           | 18                    |
| 1           | 17                    |
| 5           | 15                    |
| 10          | 10                    |
| 17.5        | 5                     |
| 23          | 0.5                   |

The following Table II gives the mechanical properties of representative Ti-Sn-Al alloys of the invention both without and with various additions of the interstitials carbon, oxygen and nitrogen. The properties are for these alloys as hot rolled to thin gauge, i. e., about 0.04 inch and thereafter annealed in argon for two hours at 850° C., unless otherwise noted.

Table II.—Mechanical properties of Ti-Sn-Al alloys with and without additions of C, O and N

| Composition, Percent<br>(Balance Titanium) |     |      |     |      | Tensile Properties: p. s. i. $\times 1,000$ |                   |                               |                              | Annealed Hardness, Vickers | Min. Bend T |
|--------------------------------------------|-----|------|-----|------|---------------------------------------------|-------------------|-------------------------------|------------------------------|----------------------------|-------------|
|                                            |     |      |     |      | 0.2% Offset Yield                           | Ultimate Strength | Percent Elonga-<br>tion in 1" | Percent Reduction<br>in Area |                            |             |
| (IODIDE TITANIUM BASE)                     |     |      |     |      |                                             |                   |                               |                              |                            |             |
| —                                          | —   | —    | —   | —    | 22                                          | 37                | 61                            | 58                           | 88                         | 0           |
| 1                                          | 1   | —    | —   | —    | 30                                          | 50                | 28                            | 55                           | 156                        | 0           |
| 1                                          | 1   | 0.25 | —   | —    | 70                                          | 79                | 25                            | 56                           | 251                        | 0.6         |
| 1                                          | 2   | —    | —   | —    | 34                                          | 53                | 29                            | 46                           | 179                        | 1.0         |
| 1                                          | 2   | 0.25 | —   | —    | 86                                          | 86                | 21                            | 53                           | 274                        | 0.5         |
| 1                                          | 3   | —    | —   | —    | 50                                          | 67                | 20                            | 48                           | 269                        | 1.5         |
| 1                                          | 3   | 0.25 | —   | —    | 95                                          | 95                | 21                            | 52                           | 327                        | 1.0         |
| 1                                          | 5   | —    | —   | —    | 67                                          | 102               | 15                            | 42                           | 278                        | 0.7         |
| 1                                          | 7.5 | —    | —   | —    | 103                                         | 106               | 20                            | 27                           | 357                        | 2.8         |
| 1.6                                        | 5   | 0.25 | —   | —    | 140                                         | 149               | 9                             | 19                           | 327                        | 4.4         |
| 2                                          | 1   | —    | —   | —    | 29                                          | 50                | 28                            | 52                           | 246                        | 0           |
| 2                                          | 1   | 0.25 | —   | —    | 71                                          | 79                | 27                            | 56                           | 238                        | 2.1         |
| 2                                          | 2   | —    | —   | —    | 41                                          | 60                | 31                            | 52                           | 273                        | 1.0         |
| 2                                          | 2   | 0.25 | —   | —    | 90                                          | 90                | 22                            | 50                           | 246                        | 1.5         |
| 2                                          | 3   | —    | —   | —    | 61                                          | 74                | 19                            | 45                           | 315                        | 1.0         |
| 2                                          | 3   | 0.25 | —   | —    | 102                                         | 103               | 19                            | 49                           | 310                        | 1.3         |
| 2                                          | 5   | —    | —   | —    | 81                                          | 93                | 18                            | 46                           | 323                        | 4.2         |
| 2                                          | 5   | 0.25 | —   | —    | 140                                         | 151               | 13                            | 42                           | 333                        | 2.2         |
| 2                                          | 5   | —    | —   | 0.06 | 96                                          | 107               | 13                            | 24                           | 392                        | 2.1         |
| 2                                          | 5   | —    | —   | 0.16 | 126                                         | 133               | 11                            | 24                           | 428                        | Br          |
| 2                                          | 5   | —    | —   | 0.24 | 139                                         | 0                 | 10                            | 10                           | 421                        | Br          |
| 2                                          | 5   | —    | —   | 0.25 | 134                                         | 1                 | 10                            | 10                           | 312                        | 1.6         |
| 2.5                                        | 5   | —    | —   | —    | 81                                          | 88                | 14                            | 43                           | 329                        | 4.2         |
| 2.5                                        | 5   | 0.25 | —   | —    | 145                                         | 157               | —                             | 15                           | 324                        | 1.8         |
| 2.5                                        | 7.5 | —    | —   | —    | 94                                          | 101               | 16                            | 42                           | 408                        | Br          |
| 2.5                                        | 10  | —    | —   | —    | 107                                         | —                 | —                             | —                            | 211                        | 1.5         |
| 3                                          | 1   | —    | —   | —    | 38                                          | 57                | 27                            | 48                           | 211                        | 1.5         |
| 3                                          | 1   | 0.25 | —   | —    | 85                                          | 90                | 19                            | 54                           | 278                        | 1.0         |
| 3                                          | 2   | —    | —   | —    | 48                                          | 63                | 21                            | 49                           | 235                        | 2.1         |
| 3                                          | 2   | 0.25 | —   | —    | 96                                          | 96                | 27                            | 55                           | 301                        | 1.0         |
| 3                                          | 3   | —    | —   | —    | 70                                          | 82                | 17                            | 44                           | 258                        | 1.5         |
| 3                                          | 3   | 0.25 | —   | —    | 108                                         | 109               | 17                            | 58                           | 329                        | 1.1         |
| 3                                          | 5   | 0.25 | —   | —    | 139                                         | 149               | 13                            | 27                           | 343                        | 4.2         |
| 3.5                                        | 5   | 0.25 | —   | —    | 144                                         | 161               | 11                            | 28                           | 355                        | 4.2         |
| 5                                          | 2   | —    | —   | —    | 60                                          | 75                | 20                            | 41                           | 250                        | 1.0         |
| 5                                          | 5   | —    | —   | —    | 90                                          | 94                | 12                            | 20                           | 312                        | 1.1         |
| 5                                          | 5   | 0.25 | —   | —    | 144                                         | 147               | 17                            | 24                           | 391                        | 2.3         |
| 5                                          | 7.5 | —    | —   | —    | 109                                         | 118               | 14                            | 26                           | 357                        | 0.7         |
| 7.5                                        | 5   | —    | —   | —    | 116                                         | 116               | —                             | 5                            | 391                        | Br          |
| 7.5                                        | 7.5 | 0.25 | —   | —    | 110                                         | 0                 | 0                             | 0                            | 398                        | 6.2         |
| 10                                         | 2   | —    | —   | —    | 85                                          | 101               | 13                            | 38                           | 302                        | 2.0         |
| 10                                         | 2   | 0.2  | —   | —    | 123                                         | 127               | 20                            | 39                           | 380                        | 1.5         |
| 10                                         | 2   | —    | 0.2 | —    | 115                                         | 123               | 15                            | 34                           | 376                        | 2.2         |
| 10                                         | 2   | —    | 0.2 | —    | 135                                         | 142               | 16                            | 30                           | 408                        | 2.1         |
| 15                                         | 2   | —    | —   | —    | 107                                         | 109               | 7                             | 26                           | 328                        | 1.7         |
| (COMMERCIAL PURITY TITANIUM BASE)          |     |      |     |      |                                             |                   |                               |                              |                            |             |
| —                                          | —   | —    | —   | —    | 49                                          | 76                | 24                            | 44                           | 197                        | 1.3         |
| 1                                          | 4   | —    | —   | —    | 87                                          | 98                | 20                            | 47                           | —                          | 1.7         |
| 1                                          | 5   | —    | —   | —    | 106                                         | 116               | 16                            | 38                           | 374                        | 2.7         |
| 2                                          | 4   | —    | —   | —    | 90                                          | 100               | 22                            | 49                           | —                          | 1.7         |
| 2                                          | 5   | —    | —   | —    | 114                                         | 122               | 18                            | 39                           | 330                        | 2.5         |
| 2.5                                        | 5   | —    | —   | —    | 106                                         | 114               | 16                            | 41                           | 353                        | 1.7         |
| 3                                          | 4   | —    | —   | —    | 97                                          | 106               | 17                            | 46                           | —                          | 2.5         |
| 3                                          | 5   | —    | —   | —    | 108                                         | 114               | 18                            | 40                           | 357                        | 3.3         |
| 3                                          | 10  | —    | —   | —    | 110                                         | —                 | 18                            | 35                           | —                          | 2.5         |
| 4                                          | 4   | —    | —   | —    | 108                                         | 116               | 21                            | 44                           | —                          | 2.5         |
| 4                                          | 5   | —    | —   | —    | 74                                          | 87                | 27                            | 44                           | 268                        | 1.8         |
| 5                                          | 1   | —    | —   | —    | 83                                          | 92                | 21                            | 58                           | 299                        | 1.7         |
| 5                                          | 2   | —    | —   | —    | 92                                          | 102               | 15                            | 28                           | 319                        | 2.8         |
| 5                                          | 3   | —    | —   | —    | 103                                         | 121               | 16                            | 24                           | 356                        | 3.6         |
| 5                                          | 3.5 | —    | —   | —    | 104                                         | 122               | 19                            | 34                           | 360                        | 2.7         |
| 5                                          | 4.5 | —    | —   | —    | 117                                         | 124               | 19                            | 49                           | 373                        | 2.2         |
| 5                                          | 5   | —    | —   | —    | 120                                         | 125               | 20                            | 47                           | 406                        | 2.5         |
| 6                                          | 3   | —    | —   | —    | 105                                         | 116               | 15                            | 38                           | 331                        | 2.8         |
| 6                                          | 4   | —    | —   | —    | 115                                         | 123               | 19                            | 42                           | 344                        | 3.4         |

Table II.—Mechanical properties of Ti-Sn-Al alloys with and without additions of C, O and N.—Continued

| Composition, Percent<br>(Balance Titanium)  |     |      |     |      |     | Tensile Properties: p. s. i. $\times 1,000$ |                      |                                  |                                 | Annealed<br>Hardness,<br>Vickers | Min. Bend<br>T |
|---------------------------------------------|-----|------|-----|------|-----|---------------------------------------------|----------------------|----------------------------------|---------------------------------|----------------------------------|----------------|
|                                             |     |      |     |      |     | 0.2%<br>Offset<br>Yield                     | Ultimate<br>Strength | Percent<br>Elonga-<br>tion in 1" | Percent<br>Reduction<br>in Area |                                  |                |
| (COMMERCIAL PURITY TITANIUM BASE)—Continued |     |      |     |      |     |                                             |                      |                                  |                                 |                                  |                |
| 6                                           | 5   | --   | --  | --   | --  | 120                                         | 121                  | 12                               | 32                              | 373                              | 3.5            |
| 7                                           | 4   | --   | --  | --   | --  | 113                                         | 118                  | 14                               | 44                              | 350                              | 3.5            |
| 9                                           | 1   | --   | --  | --   | --  | 86                                          | 99                   | 19                               | 42                              | 299                              | 1.7            |
| 9                                           | 2   | --   | --  | --   | --  | 99                                          | 109                  | 21                               | 46                              | 333                              | 2.7            |
| 9                                           | 3   | --   | --  | --   | --  | 110                                         | 118                  | 18                               | 33                              | 357                              | 2.5            |
| 9                                           | 3.5 | --   | --  | --   | --  | 120                                         | 132                  | 19                               | 33                              | 390                              | 2.5            |
| 9                                           | 4   | --   | --  | --   | --  | 125                                         | 132                  | 21                               | 40                              | 388                              | 4.6            |
| 9                                           | 4.5 | --   | --  | --   | --  | 131                                         | 131                  | 21                               | 46                              | 421                              | 2.3            |
| 9                                           | 5   | --   | --  | --   | --  | 137                                         | 137                  | 13                               | 30                              | 388                              | 3.0            |
| 10                                          | 1   | --   | --  | --   | --  | 95                                          | 104                  | 16                               | 48                              | 299                              | 3.0            |
| 10                                          | 2   | --   | --  | --   | --  | 115                                         | 122                  | 13                               | 45                              | 336                              | 4.3            |
| 10                                          | 3   | --   | --  | --   | --  | 126                                         | 131                  | 16                               | 43                              | 376                              | 3.2            |
| 13                                          | 1   | --   | --  | --   | --  | 112                                         | 122                  | 18                               | 26                              | 345                              | 2.5            |
| 13                                          | 2   | --   | --  | --   | --  | 124                                         | 124                  | 18                               | 30                              | 363                              | 2.6            |
| 13                                          | 3   | --   | --  | --   | --  | 135                                         | 135                  | 12                               | 25                              | 366                              | 5.1            |
| 13                                          | 2.5 | --   | --  | --   | --  | 134                                         | 138                  | 20                               | 36                              | 394                              | 2.5            |
| 13                                          | 4   | --   | --  | --   | --  | 143                                         | 146                  | 12                               | 27                              | 376                              | 4.8            |
| 13                                          | 4.5 | --   | --  | --   | --  | 146                                         | 149                  | 4                                | 18                              | 389                              | Br             |
| 13                                          | 5   | --   | --  | --   | --  | 163                                         | 1                    | 10                               | 422                             | Br                               |                |
| 116                                         | 1   | --   | --  | --   | --  | 97                                          | 131                  | 16                               | 21                              | 314                              | 1.8            |
| 116                                         | 2   | --   | --  | --   | --  | 133                                         | 145                  | 19                               | 30                              | 344                              | 2.4            |
| 116                                         | 3   | --   | --  | --   | --  | 152                                         | 164                  | 10                               | 19                              | 384                              | Br             |
| 116                                         | 4   | --   | --  | --   | --  | 148                                         | 1                    | 5                                | 387                             | Br                               |                |
| 119                                         | 1   | --   | --  | --   | --  | 126                                         | 147                  | 14                               | 29                              | 329                              | 1.2            |
| 119                                         | 2   | --   | --  | --   | --  | 135                                         | 151                  | 7                                | 8                               | 342                              | 2.3            |
| 119                                         | 3   | --   | --  | --   | --  | 140                                         | 154                  | 4                                | 9                               | 372                              | Br             |
| 1                                           | 4   | 0.1  | --  | --   | --  | 101                                         | 107                  | 19                               | 51                              | -----                            | 1.7            |
| 1                                           | 4   | 0.2  | --  | --   | --  | 119                                         | 120                  | 20                               | 52                              | -----                            | 1.7            |
| 1                                           | 4   | --   | 0.1 | --   | --  | 100                                         | 109                  | 17                               | 44                              | -----                            | 2.4            |
| 1                                           | 4   | --   | 0.2 | --   | --  | 115                                         | 123                  | 19                               | 42                              | -----                            | 3.4            |
| 1                                           | 4   | --   | --  | 0.1  | --  | 122                                         | 128                  | 18                               | 30                              | -----                            | 2.3            |
| 1                                           | 5   | 0.1  | --  | --   | --  | 128                                         | 133                  | 16                               | 38                              | 422                              | 5.4            |
| 1                                           | 5   | 0.2  | --  | --   | --  | 138                                         | 143                  | 14                               | 31                              | 451                              | 6.2            |
| 1                                           | 5   | 0.25 | --  | --   | --  | 139                                         | 144                  | 20                               | 40                              | 444                              | 2.5            |
| 1                                           | 5   | --   | 0.1 | --   | --  | 120                                         | 129                  | 16                               | 39                              | 393                              | 4.4            |
| 1                                           | 5   | --   | 0.2 | --   | --  | 129                                         | 136                  | 21                               | 36                              | 431                              | 5.1            |
| 1                                           | 5   | --   | --  | 0.1  | --  | 129                                         | 135                  | 14                               | 35                              | 384                              | 3.5            |
| 2                                           | 2   | 0.1  | --  | --   | --  | 104                                         | 111                  | 19                               | 48                              | -----                            | 1.6            |
| 2                                           | 2   | 0.2  | --  | --   | --  | 122                                         | 124                  | 22                               | 52                              | -----                            | 1.7            |
| 2                                           | 4   | --   | 0.1 | --   | --  | 108                                         | 117                  | 22                               | 49                              | -----                            | 1.7            |
| 2                                           | 4   | --   | 0.2 | --   | --  | 113                                         | 121                  | 18                               | 47                              | -----                            | 3.5            |
| 2                                           | 5   | 0.2  | --  | --   | 0.1 | 115                                         | 122                  | 16                               | 43                              | -----                            | 2.3            |
| 2                                           | 5   | --   | 0.1 | --   | --  | 136                                         | 141                  | 18                               | 35                              | 423                              | 4.7            |
| 2                                           | 5   | --   | 0.2 | --   | --  | 128                                         | 136                  | 12                               | 23                              | 437                              | 2.6            |
| 2                                           | 5   | --   | --  | 0.1  | --  | 127                                         | 133                  | 17                               | 34                              | 423                              | 5.1            |
| 2.5                                         | 5   | 0.1  | --  | --   | --  | 127                                         | 134                  | 16                               | 31                              | 394                              | 3.7            |
| 2.5                                         | 5   | 0.2  | --  | --   | --  | 143                                         | 147                  | 19                               | 33                              | 438                              | 6.6            |
| 2.5                                         | 5   | --   | 0.2 | --   | --  | 141                                         | 143                  | 22                               | 37                              | 422                              | 6.4            |
| 2.5                                         | 5   | --   | --  | 0.1  | --  | 137                                         | 142                  | 16                               | 39                              | 423                              | 5.2            |
| 2.5                                         | 5   | --   | --  | 0.2  | --  | 124                                         | 131                  | 3                                | 421                             | -----                            | 5.5            |
| 3                                           | 4   | 0.1  | --  | --   | --  | 151                                         | 155                  | 5                                | 15                              | 442                              | Br             |
| 3                                           | 4   | 0.2  | --  | --   | --  | 119                                         | 123                  | 20                               | 48                              | -----                            | 1.7            |
| 3                                           | 4   | --   | 0.1 | --   | --  | 125                                         | 127                  | 23                               | 49                              | -----                            | 1.7            |
| 3                                           | 4   | --   | 0.2 | --   | --  | 112                                         | 120                  | 17                               | 43                              | -----                            | 2.6            |
| 3                                           | 4   | --   | --  | 0.1  | --  | 116                                         | 124                  | 19                               | 45                              | -----                            | 3.2            |
| 3                                           | 5   | 0.1  | --  | --   | --  | 125                                         | 130                  | 18                               | 42                              | -----                            | 4.8            |
| 3                                           | 5   | 0.2  | --  | --   | --  | 138                                         | 141                  | 19                               | 33                              | 421                              | 4.8            |
| 3                                           | 5   | 0.25 | --  | --   | --  | 140                                         | 144                  | 17                               | 29                              | 421                              | 4.5            |
| 3                                           | 5   | --   | 0.1 | --   | --  | 142                                         | 144                  | 20                               | 35                              | 420                              | 2.7            |
| 3                                           | 5   | --   | 0.2 | --   | --  | 132                                         | 138                  | 16                               | 40                              | 421                              | 5.2            |
| 3                                           | 5   | --   | --  | 0.1  | --  | 139                                         | 143                  | 16                               | 31                              | 424                              | 5.1            |
| 3                                           | 5   | --   | --  | 0.2  | --  | 122                                         | 128                  | 6                                | 12                              | 392                              | 5.6            |
| 3                                           | 5   | --   | --  | 0.1  | 0.2 | 148                                         | 152                  | 5                                | 15                              | 429                              | Br             |
| 4                                           | 4   | 0.1  | --  | --   | --  | 117                                         | 121                  | 19                               | 51                              | -----                            | 2.5            |
| 4                                           | 4   | 0.2  | --  | --   | --  | 133                                         | 135                  | 15                               | 50                              | -----                            | 1.7            |
| 4                                           | 4   | --   | 0.1 | --   | --  | 119                                         | 126                  | 15                               | 40                              | -----                            | 2.5            |
| 4                                           | 4   | --   | 0.2 | --   | --  | 132                                         | 147                  | 21                               | 38                              | -----                            | 4.6            |
| 4                                           | 4   | --   | --  | 0.1  | --  | 106                                         | 109                  | 2                                | 6                               | -----                            | 3.0            |
| 4                                           | 5   | 0.1  | --  | --   | --  | 130                                         | 134                  | 20                               | 43                              | 405                              | 4.9            |
| 4                                           | 5   | --   | 0.2 | --   | --  | 136                                         | 137                  | 2                                | 15                              | 428                              | 7.0            |
| 4                                           | 5   | --   | --  | 0.1  | --  | 129                                         | 134                  | 12                               | 23                              | 404                              | 5.4            |
| 4                                           | 5   | --   | --  | 0.2  | --  | 155                                         | 156                  | 2                                | 12                              | 454                              | Br             |
| 5                                           | 1   | 0.2  | --  | --   | --  | 105                                         | 108                  | 25                               | 50                              | 322                              | 1.2            |
| 5                                           | 1   | --   | 0.2 | --   | --  | 105                                         | 106                  | 19                               | 42                              | 348                              | 3.3            |
| 5                                           | 1   | --   | --  | 0.2  | --  | 127                                         | 135                  | 21                               | 38                              | 373                              | 2.0            |
| 5                                           | 2   | 0.2  | --  | --   | --  | 118                                         | 125                  | 22                               | 49                              | 348                              | 2.4            |
| 5                                           | 2   | --   | 0.2 | --   | --  | 117                                         | 125                  | 24                               | 40                              | 333                              | 2.4            |
| 5                                           | 2   | --   | --  | 0.3  | --  | 125                                         | 132                  | 19                               | 40                              | 376                              | 2.4            |
| 5                                           | 3   | 0.2  | --  | --   | --  | 125                                         | 129                  | 20                               | 46                              | 363                              | 1.9            |
| 5                                           | 3   | --   | 0.1 | --   | --  | 125                                         | 139                  | 16                               | 31                              | 391                              | 4.8            |
| 5                                           | 3   | --   | 0.2 | --   | --  | 124                                         | 132                  | 20                               | 41                              | 390                              | 2.2            |
| 5                                           | 3   | --   | --  | 0.3  | --  | 131                                         | 147                  | 16                               | 31                              | 413                              | 6.6            |
| 5                                           | 3   | --   | --  | 0.4  | --  | 151                                         | 155                  | 6                                | 12                              | 431                              | Br             |
| 5                                           | 3   | --   | --  | 0.20 | --  | 142                                         | 146                  | 15                               | 16                              | 417                              | 2.4            |
| 9                                           | 1   | 0.2  | --  | --   | --  | 118                                         | 123                  | 23                               | 48                              | 357                              | 2.4            |
| 9                                           | 1   | --   | 0.2 | --   | --  | 107                                         | 118                  | 9                                | 11                              | 380                              | 2.3            |
| 9                                           | 1   | --   | --  | 0.15 | --  | 120                                         | 128                  | 9                                | 15                              | 373                              | 2.4            |
| 9                                           | 2   | 0.2  | --  | --   | --  | 132                                         | 136                  | 16                               | 38                              | 380                              | 2.3            |
| 9                                           | 2   | --   | 0.2 | --   | --  | 110                                         | 117                  | 5                                | 15                              | 376                              | 2.3            |
| 9                                           | 2   | --   | --  | 0.16 | --  | 131                                         | 143                  | 16                               | 20                              | 390                              | 3.2            |
| 9                                           | 3   | 0.1  | --  | --   | --  | 142                                         | 142                  | 16                               | 39                              | 401                              | 2.4            |
| 9                                           | 3   | 0.2  | --  | --   | --  | 139                                         | 142                  | 16                               | 40                              | 397                              | 3.3            |
| 9                                           | 3   | 0.3  | --  | --   | --  | 147                                         | 156                  | 23                               | 40                              | 418                              | 4.9            |
| 9                                           | 3   | 0.4  | --  | --   | --  | 161                                         | 163                  | 19                               | 32                              | 450                              | Br             |
| 9                                           | 3   | --   | 0.2 | --   | --  | 130                                         | 134                  | 17                               | 28                              | 401                              | 3.3            |
| 9                                           | 3   | --   | --  | 0.20 | --  | 148                                         | 152                  | 9                                | 14                              | -----                            | Br             |

<sup>1</sup> Annealed 2 hours at 950° C.

Table II.—Mechanical properties of Ti-Sn-Al alloys with and without additions of C, O and N—Continued

| Composition, Percent<br>(Balance Titanium)  |     |      |      |      | Tensile Properties: p. s. i. $\times 1,000$ |                      |                                  |                                 | Annealed<br>Hardness,<br>Vickers | Min. Bend<br>T |
|---------------------------------------------|-----|------|------|------|---------------------------------------------|----------------------|----------------------------------|---------------------------------|----------------------------------|----------------|
|                                             |     |      |      |      | 0.2%<br>Offset<br>Yield                     | Ultimate<br>Strength | Percent<br>Elonga-<br>tion in 1" | Percent<br>Reduction<br>in Area |                                  |                |
| Sn                                          | Al  | O    | O    | N    |                                             |                      |                                  |                                 |                                  |                |
| (COMMERCIAL PURITY TITANIUM BASE)—Continued |     |      |      |      |                                             |                      |                                  |                                 |                                  |                |
| 10                                          | 3   | 0.4  | --   | --   | 165                                         | 165                  | 8                                | 24                              | 433                              | Br             |
| 10                                          | 3   | 0.6  | --   | --   | (2)                                         | (2)                  | (2)                              | (2)                             | 455                              | Br             |
| 10                                          | 3   | 0.8  | --   | --   | (2)                                         | (2)                  | (2)                              | (2)                             | 478                              | Br             |
| 13                                          | 1   | 0.2  | --   | --   | 122                                         | 148                  | 13                               | 23                              | 390                              | 2.6            |
| 13                                          | 1   | 0.26 | --   | --   | 139                                         | 144                  | 22                               | 43                              | 333                              | 3.1            |
| 13                                          | 1   | --   | 0.2  | 0.14 | 134                                         | 140                  | 15                               | 31                              | 376                              | 3.3            |
| 13                                          | 2   | 0.2  | --   | --   | 149                                         | 151                  | 16                               | 35                              | 413                              | 3.3            |
| 13                                          | 2   | --   | 0.2  | --   | 143                                         | 153                  | 18                               | 20                              | 411                              | 4.7            |
| 13                                          | 2   | --   | 0.2  | --   | 140                                         | 150                  | 4                                | 5                               | 356                              | 3.5            |
| 13                                          | 2   | --   | 0.16 | --   | 134                                         | 154                  | 9                                | 23                              | 357                              | 3.6            |
| 13                                          | 3   | 0.2  | --   | --   | 164                                         | 164                  | 12                               | 13                              | 416                              | Br             |
| 13                                          | 3   | --   | 0.2  | --   | 156                                         | 159                  | 5                                | 13                              | 420                              | Br             |
| 13                                          | 3   | --   | 0.22 | --   | --                                          | 166                  | 0                                | 4                               | 331                              | Br             |
| 10                                          | 2.5 | 0.2  | --   | --   | 140                                         | 141                  | 6                                | 29                              | 395                              | 5.5            |
| 10                                          | 3   | 0.2  | --   | --   | 136                                         | 146                  | 15                               | 40                              | 333                              | 2.8            |

\* Very brittle.

It is thus apparent that the ternary alloys of titanium with aluminum and tin, with or without additions of the interstitials, constitute an outstandingly versatile and desirable group, offering a wide range of properties and a composition tolerance for any given set of properties which greatly facilitates their production.

The alloys of this invention, in general, will withstand

25 Moreover, these titanium-aluminum-tin alloys are susceptible to a variety of useful modifications by additions of one or more of the various other metals above mentioned.

For example, the following Table III shows the effect 30 on mechanical properties of additions of the various alpha promoters:

| Composition, Percent (Balance<br>Titanium) |     |       |         | Tensile Properties: p. s. i. $\times 1,000$ |                      |                                |                                 | VHN | Min.<br>Bend<br>T |  |
|--------------------------------------------|-----|-------|---------|---------------------------------------------|----------------------|--------------------------------|---------------------------------|-----|-------------------|--|
|                                            |     |       |         | 0.2%<br>Offset<br>Yield                     | Ultimate<br>Strength | Percent<br>Elongation<br>in 1" | Percent<br>Reduction<br>in Area |     |                   |  |
| Sn                                         | Al  | Other | C, O, N |                                             |                      |                                |                                 |     |                   |  |
| (IODIDE TITANIUM BASE)                     |     |       |         |                                             |                      |                                |                                 |     |                   |  |
| 2.5                                        | 5   | Sb    |         |                                             |                      |                                |                                 |     |                   |  |
| 2.5                                        | 5   | 0.5   | 0.25 C  | 150                                         | 157                  | 14                             | 23                              | 300 | 4.1               |  |
| 2.5                                        | 5   | 1.0   | 0.25 C  | 137                                         | 138                  | 17                             | 26                              | 403 | 2.1               |  |
| 2.5                                        | 5   | 1.5   | 0.25 C  | 143                                         | 144                  | 5                              | 11                              | 418 | Br                |  |
| 2.5                                        | 5   | 2.5   | 0.25 C  | 142                                         | 143                  | 3                              | 9                               | 392 | Br                |  |
| 2.5                                        | 5   | 5     | 0.25 C  | -----                                       | 134                  | 1                              | 5                               | 409 | Br                |  |
| 2.5                                        | 5   | B1    |         |                                             |                      |                                |                                 |     |                   |  |
| 2.5                                        | 5   | 0.5   | 0.25 C  | 131                                         | 133                  | 15                             | 28                              | 403 | 4.1               |  |
| 2.5                                        | 5   | 1     | 0.25 C  | 132                                         | 133                  | 23                             | 36                              | 387 | 2.3               |  |
| 2.5                                        | 5   | 1.5   | 0.25 C  | 141                                         | 143                  | 3                              | 10                              | 415 | Br                |  |
| 2.5                                        | 5   | Ag    |         |                                             |                      |                                |                                 |     |                   |  |
| 2.5                                        | 5   | 0.5   | 0.25 C  | 130                                         | 132                  | 22                             | 45                              | 382 | 1.6               |  |
| 2.5                                        | 5   | 1     | 0.25 C  | 132                                         | 133                  | 20                             | 45                              | 383 | 2.3               |  |
| (COMMERCIAL PURITY TITANIUM BASE)          |     |       |         |                                             |                      |                                |                                 |     |                   |  |
| 2.5                                        | 2.5 | Sb    |         |                                             |                      |                                |                                 |     |                   |  |
| 5                                          | 2.5 | 5     | -----   | 110                                         | 115                  | 15                             | 48                              | 330 | 2.6               |  |
| 7.5                                        | 2.5 | 2.5   | -----   | 114                                         | 118                  | 13                             | 44                              | 343 | 2.8               |  |
| 2.5                                        | 2.5 | 7.5   | 0.2 C   | 110                                         | 117                  | 15                             | 40                              | 345 | 2.6               |  |
| 5                                          | 2.5 | 5     | 0.2 C   | 154                                         | 157                  | 5                              | 18                              | 400 | 6.2               |  |
| 7.5                                        | 2.5 | 2.5   | 0.2 C   | 144                                         | 146                  | 5                              | 21                              | 390 | 3.0               |  |
| 0.5                                        | 5   | 2     | -----   | 103                                         | 109                  | 15                             | 43                              | 351 | 2.8               |  |
| 1                                          | 5   | 1.5   | -----   | 106                                         | 113                  | 15                             | 37                              | 346 | 2.1               |  |
| 1.5                                        | 5   | 1     | -----   | 103                                         | 112                  | 17                             | 46                              | 343 | 2.9               |  |
| 2                                          | 5   | 0.5   | -----   | 100                                         | 111                  | 14                             | 43                              | 348 | 2.8               |  |
| 0.5                                        | 5   | 2     | 0.2 C   | (1)                                         | (1)                  | (1)                            | (1)                             | (1) | (1)               |  |
| 1                                          | 5   | 1.5   | 0.2 C   | 132                                         | 135                  | 17                             | 42                              | 394 | 2.8               |  |
| 1.5                                        | 5   | 1     | 0.2 C   | 131                                         | 135                  | 17                             | 48                              | 396 | 2.8               |  |
| 2                                          | 5   | 0.5   | 0.2 C   | 130                                         | 134                  | 7                              | 28                              | 391 | 2.8               |  |

\* Cracked during forging.

prolonged aging at temperatures as high as 400° C. without material embrittlement. Hence, they are particularly adapted for use under high temperature conditions.

The effect on mechanical properties of adding the various beta promoters is shown by the following Table IV:

Table IV

(Ti-Sn-Al BASE PLUS BETA PROMOTERS)

| Composition, Percent (Balance Titanium) |     |       |         | Tensile Properties: p. s. i. $\times 1,000$ |                   |                          |                           | Min. VHN | Min. Bend T |         |
|-----------------------------------------|-----|-------|---------|---------------------------------------------|-------------------|--------------------------|---------------------------|----------|-------------|---------|
| Sn                                      | Al  | Other | C, O, N | 0.2% Offset Yield                           | Ultimate Strength | Percent Elongation in 1" | Percent Reduction in Area |          |             |         |
| (IODIDE TITANIUM BASE)                  |     |       |         |                                             |                   |                          |                           |          |             |         |
| 2.5                                     | 5   | Mn    | 0.5     | 0.25 C                                      | 133               | 133                      | 11                        | 21       | 411         | 3.4     |
| 2.5                                     | 5   |       | 1       | 0.25 C                                      | 136               | 138                      | 13                        | 16       | 423         | 4.0     |
| 2.5                                     | 5   |       | 1.5     | 0.25 O                                      | 151               | 152                      | 12                        | 12       | 438         | Br      |
| 2.5                                     | 5   | Be    | 0.1     | 0.25 C                                      | 133               | 133                      | 22                        | 32       | 396         | 4.0     |
| 2.5                                     | 5   |       | 0.25    | 0.25 O                                      | 137               | 139                      | 10                        | 19       | 409         | 3.8     |
| 2.5                                     | 5   | Cu    | 0.5     | 0.25 O                                      | 144               | 156                      | 12                        | 21       | 404         | 4.1     |
| 2.5                                     | 5   |       | 1       | 0.25 C                                      | 133               | 133                      | 11                        | 32       | 407         | 2.5     |
| 2.5                                     | 5   |       | 1.5     | 0.25 C                                      | 134               | 134                      | 10                        | 24       | 424         | 3.6     |
| 2.5                                     | 5   | Zr    | 0.5     | 0.25 C                                      | 129               | 132                      | 19                        | 36       | 377         | 2.3     |
| 2.5                                     | 5   |       | 1       | 0.25 O                                      | 137               | 138                      | 21                        | 41       | 391         | 4.5     |
| (COMMERCIAL PURITY TITANIUM BASE)       |     |       |         |                                             |                   |                          |                           |          |             |         |
| 5                                       | 2   | Mn    | 4       | -----                                       | 116               | 126                      | 12                        | 45       | 443         | 2.5     |
| 5                                       | 2   |       | 5       | -----                                       | 140               | 145                      | 5                         | 26       | 389         | 4.5     |
| 10                                      | 1   |       | 0.5     | -----                                       | 107               | 114                      | 13                        | 48       | 318         | 2.6     |
| 10                                      | 1   |       | 1       | -----                                       | 111               | 118                      | 11                        | 42       | 326         | 3.6     |
| 10                                      | 1   |       | 1.5     | -----                                       | 120               | 127                      | 14                        | 42       | 335         | 2.9     |
| 10                                      | 1   |       | 2       | -----                                       | 128               | 134                      | 11                        | 41       | 335         | 2.8     |
| 10                                      | 1   |       | 3       | -----                                       | 138               | 145                      | 11                        | 35       | 383         | 2.0     |
| 10                                      | 2   |       | 0.5     | -----                                       | 108               | 118                      | 12                        | 41       | 338         | 6.6     |
| 10                                      | 2   |       | 1       | -----                                       | 139               | 143                      | 11                        | 40       | 359         | 3.2/6.2 |
| 10                                      | 2   |       | 1.5     | -----                                       | 138               | 143                      | 12                        | 37       | 361         | 3.7     |
| 10                                      | 2   |       | 2       | -----                                       | 153               | 158                      | 8                         | 32       | 372         | 3.5/6.0 |
| 10                                      | 2   |       | 3       | -----                                       | 164               | 164                      | 14                        | 47       | 404         | 2.2     |
| 10                                      | 2   |       | 4       | -----                                       | 146               | 154                      | 11                        | 38       | 382         | 1.5     |
| 10                                      | 3   |       | 0.5     | -----                                       | 147               | 150                      | 9                         | 25       | 327         | 7.2     |
| 10                                      | 3   |       | 1       | -----                                       | 143               | 149                      | 13                        | 34       | 333         | 4.0     |
| 10                                      | 3   |       | 1.5     | -----                                       | 160               | 154                      | 11                        | 22       | 339         | Br      |
| 10                                      | 3   |       | 2       | -----                                       | 168               | 172                      | 7                         | 22       | 360         | 6.7/Br  |
| 10                                      | 3   |       | 3       | -----                                       | 179               | 181                      | 10                        | 34       | 414         | 2.5     |
| 10                                      | 1   |       | 5       | -----                                       | 149               | 156                      | 10                        | 41       | 411         | 1.5     |
| 10                                      | 2   |       | 5       | -----                                       | 162               | 167                      | 7                         | 13       | 412         | 1.8     |
| 10                                      | 3   |       | 5       | -----                                       | 181               | 187                      | 2                         | 8        | 457         | 6.2     |
| 10                                      | 1   |       | 7       | -----                                       | 154               | 164                      | 8                         | 33       | 416         | 2.5     |
| 10                                      | 2   |       | 7       | -----                                       | 184               | 186                      | 5                         | 12       | 443         | 6.5     |
| 10                                      | 3   |       | 0.1     | -----                                       | 116               | 126                      | 16                        | 45       | 362         | 4.4     |
| 10                                      | 3   |       | 0.3     | -----                                       | 112               | 119                      | 12                        | 46       | 342         | 4.4     |
| 10                                      | 3   |       | 0.5     | -----                                       | 122               | 132                      | 14                        | 41       | 344         | 4.3     |
| 5                                       | 2   | Mo    | 5       | -----                                       | 124               | 130                      | 12                        | 43       | 338         | 2.0     |
| 10                                      | 2   |       | 5       | -----                                       | 142               | 150                      | 13                        | 24       | 350         | 2.6     |
| 15                                      | 2   |       | 5       | -----                                       | 192               | 195                      | 1                         | 4        | 402         | Br      |
| 10                                      | 1   |       | 2.5     | -----                                       | 130               | 136                      | 14                        | 46       | 355         | 1.5     |
| 10                                      | 2   |       | 2.5     | -----                                       | 142               | 150                      | 13                        | 41       | 358         | 2.6     |
| 10                                      | 3   |       | 2.5     | -----                                       | 173               | 178                      | 8                         | 35       | 397         | 5.0     |
| 10                                      | 4   |       | 2.5     | -----                                       | 177               | 177                      | 1                         | 2        | 435         | 4.8     |
| 10                                      | 1   |       | 5       | -----                                       | 134               | 140                      | 11                        | 32       | 329         | 2.2     |
| 10                                      | 2   | Mo    | 5       | -----                                       | 138               | 153                      | 13                        | 24       | 350         | 2.1     |
| 10                                      | 3   |       | 5       | -----                                       | 171               | 174                      | 4                         | 19       | 378         | 2.0     |
| 10                                      | 4   |       | 5       | -----                                       | 113               | 113                      | 1                         | 2        | 431         | Br      |
| 10                                      | 1   |       | 10      | -----                                       | 130               | 135                      | 9                         | 38       | 320         | 0       |
| 10                                      | 2   |       | 10      | -----                                       | 148               | 154                      | 9                         | 25       | 332         | 1.7     |
| 10                                      | 3   |       | 10      | -----                                       | 174               | 180                      | 3                         | 12       | 387         | 5.3     |
| 10                                      | 4   |       | 10      | -----                                       | 161               | 161                      | 1                         | 3        | 416         | Br      |
| 10                                      | 1   |       | 0.5     | -----                                       | 125               | 130                      | 11                        | 46       | -----       | 2.8/5.7 |
| 10                                      | 1   |       | 1       | -----                                       | 131               | 136                      | 15                        | 42       | -----       | 3.7/5.5 |
| 10                                      | 1   |       | 1.5     | -----                                       | 131               | 136                      | 12                        | 45       | -----       | 2.8     |
| 10                                      | 2   |       | 2       | -----                                       | 132               | 139                      | 8                         | 39       | -----       | 2.8     |
| 10                                      | 2   |       | 0.5     | -----                                       | 149               | 154                      | 9                         | 36       | -----       | Br      |
| 10                                      | 2   |       | 1       | -----                                       | 147               | 153                      | 14                        | 42       | -----       | Br      |
| 10                                      | 2   |       | 1.5     | -----                                       | 155               | 160                      | 7                         | 29       | -----       | Br      |
| 10                                      | 2   |       | 2       | -----                                       | 156               | 161                      | 9                         | 32       | -----       | 5.0/Br  |
| 10                                      | 3   |       | 0.5     | -----                                       | 161               | 163                      | 7                         | 35       | -----       | 5.5/Br  |
| 10                                      | 3   |       | 1       | -----                                       | 165               | 169                      | 3                         | 14       | -----       | Br      |
| 10                                      | 3   |       | 1.5     | -----                                       | 167               | 169                      | 3                         | 19       | -----       | Br      |
| 10                                      | 3   |       | 2       | -----                                       | 176               | 176                      | 5                         | 16       | -----       | Br      |
| 0.5                                     | 0.5 | 30    | 30      | -----                                       | 124               | 125                      | 5                         | 28       | 282         | 0.4     |
| 5                                       | 2   | Cr    | 4       | -----                                       | 142               | 147                      | 15                        | 34       | 363         | 2.1     |
| 10                                      | 2   |       | 4       | -----                                       | 155               | 164                      | 10                        | 30       | 366         | 2.5     |
| 15                                      | 2   |       | 4       | -----                                       | 192               | 202                      | 1                         | 3        | 419         | Br      |
| 10                                      | 1   |       | 2       | -----                                       | 135               | 141                      | 14                        | 45       | 346         | 1.8     |
| 10                                      | 2   |       | 2       | -----                                       | 147               | 153                      | 13                        | 44       | 360         | 2.5     |
| 10                                      | 3   |       | 2       | -----                                       | 179               | 182                      | 10                        | 28       | 385         | 2.0     |
| 10                                      | 4   |       | 2       | -----                                       | 193               | 198                      | 4                         | 5        | 415         | 5.3     |
| 10                                      | 1   |       | 4       | -----                                       | 138               | 147                      | 13                        | 35       | 360         | 1.7     |
| 10                                      | 2   |       | 4       | -----                                       | 155               | 164                      | 10                        | 30       | 366         | 1.9     |
| 10                                      | 3   |       | 4       | -----                                       | 180               | 185                      | 9                         | 26       | 407         | 2.7     |
| 10                                      | 4   |       | 4       | -----                                       | 200               | 204                      | 1                         | 2        | 447         | Br      |
| 10                                      | 1   |       | 8       | -----                                       | 137               | 147                      | 13                        | 28       | 343         | 0.8     |
| 10                                      | 2   |       | 8       | -----                                       | 169               | 167                      | 9                         | 25       | 378         | 3.7     |

Table IV.—Continued

| Composition, Percent (Balance Titanium)     |     |       |         | Tensile Properties: p. s. i. $\times 1,000$ |                   |                          |                           | VHN   | Min. Bend T |
|---------------------------------------------|-----|-------|---------|---------------------------------------------|-------------------|--------------------------|---------------------------|-------|-------------|
| Sn                                          | Al  | Other | C, O, N | 0.2% Offset Yield                           | Ultimate Strength | Percent Elongation in 1" | Percent Reduction in Area |       |             |
| (COMMERCIAL PURITY TITANIUM BASE)—Continued |     |       |         |                                             |                   |                          |                           |       |             |
| 10                                          | 3   | 8     | -----   | (1)                                         | (1)               | (1)                      | (1)                       | (1)   | (1)         |
| 10                                          | 4   | 8     | -----   | (1)                                         | (1)               | (1)                      | (1)                       | (1)   | 2.9         |
| 10                                          | 1   | 0.5   | -----   | 124                                         | 129               | 17                       | 40                        | ----- | 2.9         |
| 10                                          | 1   | 1     | -----   | 131                                         | 136               | 12                       | 42                        | ----- | 2.9         |
| 10                                          | 1   | 1.5   | -----   | 135                                         | 140               | 14                       | 16                        | ----- | 3.4         |
| 10                                          | 2   | 0.5   | -----   | 115                                         | 123               | 15                       | 43                        | ----- | 3.4         |
| 10                                          | 2   | 1     | -----   | 131                                         | 137               | 10                       | 36                        | ----- | 4.8         |
| 10                                          | 2   | 1.5   | -----   | 139                                         | 146               | 8                        | 23                        | ----- | 5.7         |
| 10                                          | 3   | 0.5   | -----   | 122                                         | 129               | 13                       | 35                        | ----- | 5.3         |
| 10                                          | 3   | 1     | -----   | 143                                         | 149               | 7                        | 24                        | ----- | 5.2/Br      |
| 10                                          | 3   | 1.5   | -----   | 141                                         | 149               | 8                        | 21                        | ----- | 5.5/Br      |
|                                             |     | Fe    |         |                                             |                   |                          |                           |       |             |
| 10                                          | 1   | 0.5   | -----   | 103                                         | 116               | 21                       | 45                        | 331   | 2.7         |
| 10                                          | 1   | 1     | -----   | 118                                         | 136               | 15                       | 34                        | 356   | 2.4         |
| 10                                          | 1   | 1.5   | -----   | 122                                         | 136               | 16                       | 37                        | 365   | 2.8         |
| 10                                          | 1   | 2     | -----   | 150                                         | 161               | 14                       | 31                        | 357   | 2.3         |
| 10                                          | 2   | 0.5   | -----   | 118                                         | 132               | 16                       | 41                        | 363   | 2.8         |
| 10                                          | 2   | 1     | -----   | 127                                         | 144               | 14                       | 32                        | 371   | 2.6         |
| 10                                          | 2   | 1.5   | -----   | 136                                         | 147               | 14                       | 37                        | 388   | 4.0         |
| 10                                          | 2   | 2     | -----   | 150                                         | 165               | 11                       | 36                        | 400   | 5.1         |
| 10                                          | 3   | 0.5   | -----   | 143                                         | 151               | 16                       | 41                        | 389   | 7.9         |
| 10                                          | 3   | 1     | -----   | 142                                         | 152               | 10                       | 36                        | 400   | 2.8         |
| 10                                          | 3   | 1.5   | -----   | 169                                         | 177               | 5                        | 12                        | 395   | 2.9         |
| 10                                          | 3   | 2     | -----   | 159                                         | 167               | 9                        | 13                        | 404   | 2.8         |
| 10                                          | 4   | 2     | -----   | 189                                         | 193               | 7                        | 14                        | 441   | 5.1         |
| 10                                          | 4   | 4     | -----   | 162                                         | 173               | 9                        | 30                        | 462   | 2.3         |
| 10                                          | 2   | 4     | -----   | 158                                         | 158               | 1                        | 5                         | 433   | 6.8         |
| 10                                          | 3   | 4     | -----   | 177                                         | 177               | 1                        | 5                         | 447   | 6.7         |
| 10                                          | 4   | 4     | -----   | 63                                          | 0                 | 0                        | 0                         | 468   | 8.0         |
| 5                                           | 2   | 2     | -----   | 124                                         | 135               | 15                       | 38                        | 351   | 1.6         |
| 15                                          | 2   | 2     | (2)     | (2)                                         | (2)               | (2)                      | (2)                       | (2)   | (2)         |
| 10                                          | 3   | 0.1   | -----   | 111                                         | 120               | 13                       | 44                        | 327   | 4.4         |
| 10                                          | 3   | 0.3   | -----   | 111                                         | 122               | 15                       | 44                        | 337   | 4.4         |
| 10                                          | 3   | 0.5   | -----   | 112                                         | 125               | 15                       | 45                        | 343   | 4.4         |
|                                             |     | V     |         |                                             |                   |                          |                           |       |             |
| 10                                          | 1   | 1.5   | -----   | 118                                         | 127               | 17                       | 30                        | 358   | 4.1         |
| 10                                          | 1   | 3     | -----   | 133                                         | 139               | 14                       | 25                        | 358   | 4.4         |
| 10                                          | 1   | 5     | -----   | 136                                         | 146               | 12                       | 18                        | 364   | 2.5         |
| 10                                          | 2   | 1.5   | -----   | 118                                         | 126               | 12                       | 24                        | 372   | 4.9         |
| 10                                          | 2   | 3     | -----   | 156                                         | 165               | 5                        | 20                        | 392   | 5.6         |
| 10                                          | 2   | 5     | -----   | 168                                         | 163               | 15                       | 39                        | 394   | 4.9         |
| 10                                          | 3   | 1.5   | -----   | 133                                         | 137               | 14                       | 32                        | 385   | 4.7         |
| 10                                          | 3   | 3     | -----   | 161                                         | 165               | 14                       | 27                        | 413   | 5.2         |
| 10                                          | 3   | 5     | -----   | 172                                         | 177               | 6                        | 16                        | 391   | 5.0         |
| 0.5                                         | 0.5 | 30    | -----   | 102                                         | 107               | 15                       | 21                        | 235   | 0.4         |
|                                             |     | Zr    |         |                                             |                   |                          |                           |       |             |
| 0.5                                         | 0.5 | 30    | -----   | 122                                         | 148               | 2                        | 2                         | 308   | 6.2         |
|                                             |     | Ob    |         |                                             |                   |                          |                           |       |             |
| 0.5                                         | 0.5 | 30    | -----   | 67                                          | 88                | 14                       | 35                        | 206   | 0.5         |
| 0.5                                         | 0.5 | Ta    | -----   | 70                                          | 103               | 11                       | 18                        | 216   | 0           |

<sup>1</sup> Broke while machining tensile specimens.<sup>2</sup> Could not be fabricated.

The effect of addition of a multiplicity of beta promoters is shown in the following Table V:

Table V  
(Ti-Sn-Al BASE PLUS MULTIPLE BETA PROMOTER ADDITIONS  
[Commercial purity titanium base]

| Composition, Percent (Balance Titanium) | Tensile Properties: p. s. i. $\times 1,000$ |                   |                          |                           | VHN   | Min. Bend T |
|-----------------------------------------|---------------------------------------------|-------------------|--------------------------|---------------------------|-------|-------------|
|                                         | 0.2% Offset Yield                           | Ultimate Strength | Percent Elongation in 1" | Percent Reduction in Area |       |             |
| 10Sn-2Al-1.5Fe-4.5Mn                    | 165                                         | 168               | 4                        | 9                         | 425   | Br          |
| 10Sn-2Al-1.5Fe-2.5Mo                    | 163                                         | 169               | 8                        | 25                        | 397   | 2.8         |
| 10Sn-2Al-1.5Fe-2.5Cr                    | 157                                         | 165               | 12                       | 23                        | 387   | 2.6         |
| 10Sn-2Al-4.5Mn-2.5Mo                    | 163                                         | 172               | 10                       | 31                        | 390   | 2.5         |
| 10Sn-2Al-4.5Mn-2.5Cr                    | 159                                         | 165               | 9                        | 27                        | 383   | 2.8         |
| 10Sn-2Al-2.5Mo-2.5Cr                    | 158                                         | 171               | 8                        | 16                        | 397   | 2.5         |
| 3.6Sn-3.2Al-1.5Mo-1.5Cr                 | 128                                         | 130               | 16                       | 50                        | ----- | 3.7         |
| 4.6Sn-3.3Al-1.8Mo-1.6Cr                 | 136                                         | 138               | 16                       | 45                        | ----- | 1.4         |
| 3Sn-3Al-2Cr-2V                          | 136                                         | 138               | 11                       | 45                        | ----- | 2.9         |
| 3Sn-3Al-2Cr-2V                          | 134                                         | 149               | 14                       | 35                        | ----- | 2.9         |

It will be seen from comparison of the data given in the above Tables III-V inc. with that given in Table II, that the addition of one or more metals of the alpha promoting, beta promoting and compound forming groups, to the Ti-Sn-Al base alloy of any given analysis, results in an increase in tensile strength. For certain additions, such for example as bismuth, silver or copper, the enhancement in strength is relatively slight per percent of such alloying addition, i. e., on the order of a few percent. For other additions the enhancement in tensile strength per percent of the alloying addition is relatively great, on the order of 5 to 30% or more, as in the case of such additions as antimony, beryllium, manganese, molybdenum, chromium, iron and vanadium, etc. Moreover as further shown by the test results, the degree to which the base alloy is thus strengthened varies considerably with the amount of tin and/or aluminum present in the base alloy.

Thus, by way of illustration of the points above noted, the comparative data in the tables referred to, shows that the addition of 1% of bismuth, silver or copper to the Ti-2.5Sn-Al-0.25C base alloy, increases the tensile strength from about 130,000 to 133,000 p. s. i., an increase of about 2% per percent of alloying addition. On the other hand the addition of 1.5% Sb to the Ti-1Sn-5Al base increases the tensile strength from 116,000 to 135,000 p. s. i., an increase of about 11% in tensile strength per percent of the antimony addition. Similarly for the Ti-5Sn-2Al base, the tensile strength of which is 92,000 p. s. i., the addition of 4% manganese increases this value to 126,000 p. s. i., the addition of 5% molybdenum increases it to 130,000 p. s. i., and the addition of 4% chromium provides an increase to 147,000 p. s. i. The tensile strength is thus increased by about 8 to 15% per percent of alloy addition for such elements. On the other hand the addition of 1% manganese, molybdenum or chromium to the Ti-10Sn-1Al base increases the tensile strengths about 11% in the case of manganese and about 31% in the case of molybdenum and chromium, namely from 104,000 p. s. i. to 118,000, 136,000 and 136,000 p. s. i., respectively. Generally similar results are obtainable by vanadium additions as shown by the addition of 1.5% vanadium to the Ti-10Sn-1Al base resulting in an increase in tensile strength from 104,000 to 127,000 p. s. i., an increase of about 15% per percent of vanadium addition. Iron likewise has a high strengthening effect as shown by the addition of 2% Fe to this base resulting in an increase in tensile strength from 104,000 to 161,000 p. s. i., an increase of about 28% in tensile strength per percent of iron addition.

The above comparisons are merely illustrative of the fact above stated that additions of other metals from the groups referred to, to the Ti-Sn-Al base in general produce pronounced enhancement of the tensile strength of the resulting alloy. And this is accomplished without any material reduction in the ductility of the alloys as shown by the values for the percent elongation and minimum bend ductilities as tabulated in the various tables referred to. In this latter connection, it should be pointed out that where the alloys are to be used in sheet form, as in foils for airplane wings and the like, the minimum bend ductility may range as high as about 20 T; and where the alloys are to be used in massive form, as in forgings, the tensile elongations may range as low as 1 or 2%.

The alloys of the invention may be made by arc melting in a cold mold furnace in an inert or argon atmosphere or by other procedures.

Tests in the arc welding of alloys in accordance with the invention establish that those which are predominantly alpha in structure and some of those containing beta stabilizers, notably chromium and molybdenum, may be welded without impairment of their annealed strength and ductility characteristics. Thus, arc welded specimens of the Ti-1Sn-3Al alloy were found to have in the weld zone an ultimate strength of 88,000 p. s. i., an elongation

5  
10  
15  
20  
25  
30  
35  
40  
45

of 14%, an area reduction of 48%, a minimum bend T of 1.5 longitudinal and 3.0 transverse. Similarly the Ti-9Sn-3Al alloy had in the weld zone an ultimate strength of 125,000 p. s. i., an elongation of 10%, an area reduction of 38%, a minimum bend T of 2.5 longitudinal and 4.5 transverse. In addition, minimum bend tests made on arc welded specimens of various analyses, establish that, in general, the bend ductility in the weld zone is as good or better than that of the base metal. These conclusions are substantiated by the following test results of Table VI:

Table VI

| Composition, Per-cent (Balance Titanium) |    |       | Minimum Bend T (Longitudinal) |                 |
|------------------------------------------|----|-------|-------------------------------|-----------------|
| Sn                                       | Al | Other | Welded Sample                 | Unwelded Sample |
| 1                                        | 5  | ----- | 0.2                           | 0.2             |
| 2                                        | 5  | ----- | 1.8                           | 2.7             |
| 3                                        | 5  | ----- | 2.7                           | 2.5             |
| 4                                        | 5  | ----- | 1.8                           | 3.3             |
| 5                                        | 5  | ----- | 1.7                           | 5.7             |
| 5                                        | 2  | ----- | 0.2                           | 0.9             |
| 5                                        | 3  | ----- | 1.9                           | 1.7             |
| 5                                        | 5  | ----- | 1.6                           | 1.8             |
| 10                                       | 1  | ----- | 2.5                           | 2.5             |
| 10                                       | 1  | ----- | 1.4                           | 1.4             |
| 10                                       | 2  | ----- | 1.5                           | 1.7             |
| 10                                       | 2  | ----- | 2.0                           | 2.7             |
| 9                                        | 4  | ----- | 4.4                           | 4.6             |
| 9                                        | 5  | ----- | 5.0                           | 3.0             |
| 13                                       | 1  | ----- | 0.9                           | 1.4             |
| 13                                       | 1  | ----- | 2.5                           | 2.3             |
| 13                                       | 3  | ----- | 2.5                           | 2.3             |
| 10                                       | 1  | 4Cr   | 5.3                           | 1.7             |
| 10                                       | 2  | 4Cr   | 7.0                           | 2.5             |
| 10                                       | 2  | 5Mo   | 2.7                           | 2.2             |
| 10                                       | 2  | 5Mo   | 7.1                           | 2.1             |
| 10                                       | 1  | 10Mo  | 0.9                           | 0               |
| 10                                       | 2  | 10Mo  | 4.8                           | 1.7             |
| 5                                        | 2  | 5Mo   | 7.0                           | 2.0             |
| 10                                       | 1  | 3Mn   | 6.0                           | 2.0             |

In the appended claims: by the expression "other alpha promoters" is meant elements of the group Sb, In, Ag, Bi, Pb, Cd, Zn and Th; by the expression "beta promoters" is meant elements of the group Mo, V, Cr, Ta, Zr, Mn, Cr, Fe, W, Ni, Co and Cu; and by the expression "compound formers" is meant elements of the group Si, Be, Ce, B, As, S, Te and P.

What is claimed is:

1. An alloy consisting essentially of about: 1 to 23% tin, 0.25 to 8% aluminum, up to 1% carbon, up to 0.5% oxygen, up to 0.4% nitrogen, 0.5 to 20% of at least one other alpha promoter, balance titanium, characterized in having an ultimate strength substantially in excess of that of the corresponding base alloy without such other alpha promoter addition, said alloy also having a minimum bend ductility of not over 20 T.
2. An alloy consisting essentially of about: 1 to 23% tin, 0.25 to 8% aluminum, up to 1% carbon, up to 0.5% oxygen, up to 0.4% nitrogen, 0.5 to 50% of at least one beta promoter, balance titanium, characterized in having an ultimate strength substantially in excess of the corresponding base alloy without such beta promoter addition, said alloy also having a minimum bend ductility of not over 20 T.
3. An alloy consisting essentially of about: 1 to 23% tin, 0.25 to 8% aluminum, up to 1% carbon, up to 0.5% oxygen, up to 0.4% nitrogen, 0.5 to 20% of at least one other alpha promoter, 0.5 to 50% of at least one beta promoter, balance titanium, characterized in having an ultimate strength substantially in excess of the corresponding base alloy without such other alpha promoter and beta promoter additions, said alloy also having a minimum bend ductility of not over 20 T.
4. An alloy consisting essentially of about: 1 to 23% tin, 0.25 to 8% aluminum, up to 1% carbon, up to 0.5% oxygen, up to 0.4% nitrogen, 0.1 to 3% of at least one compound former, balance titanium, characterized in

having an ultimate strength substantially in excess of that of the corresponding base alloy without such compound former addition, and a minimum bend ductility of not over 20 T.

5. An alloy consisting essentially of about: 1 to 23% tin, 0.25 to 8% aluminum, up to 1% carbon, up to 0.5% oxygen, up to 0.4% nitrogen, 0.5 to 20% of at least one other alpha promoter, 0.5 to 50% of at least one beta promoter, 0.1 to 3% of at least one compound former, balance titanium, characterized in having an ultimate strength substantially in excess of the corresponding base alloy without such other alpha promoter, beta promoter and compound former additions, said alloy also having a minimum bend ductility of not over 20 T.

6. An alloy consisting of about: 1 to 23% tin, 0.25 to 8% aluminum, up to 1% carbon, up to 0.5% oxygen, up to 0.4% nitrogen, 0.5 to 20% of at least one other alpha promoter, balance titanium.

7. An alloy consisting of about: 1 to 23% tin, 0.25 to 8% aluminum, up to 1% carbon, up to 0.5% oxygen, up to 0.4% nitrogen, 0.5 to 50% of at least one beta promoter, balance titanium.

8. An alloy consisting of about: 1 to 23% tin, 0.25 to 8% aluminum, up to 1% carbon, up to 0.5% oxygen, up to 0.4% nitrogen, 0.5 to 20% of at least one other alpha promoter, 0.5 to 50% of at least one beta promoter, balance titanium.

9. An alloy consisting of about: 1 to 23% tin, 0.25 to 8% aluminum, up to 1% carbon, up to 0.5% oxygen, up to 0.4% nitrogen, 0.1 to 3% of at least one compound former, balance titanium.

10. An alloy consisting of about: 1 to 23% tin, 0.25 to 8% aluminum, up to 1% carbon, up to 0.5% oxygen, up to 0.4% nitrogen, 0.5 to 20% of at least one other alpha promoter, 0.5 to 50% of at least one beta promoter, 0.1 to 3% of at least one compound former, balance titanium.

11. An alloy consisting essentially of about: 1 to 23% tin, 0.25 to 8% aluminum, up to 1% carbon, up to 0.5% oxygen, up to 0.4% nitrogen, 0.5 to 50% of at least one additional element selected from the group consisting of molybdenum, vanadium, columbium, tantalum, zirconium, balance titanium, characterized in having an ultimate strength substantially in excess of that of the corresponding base alloy without such addition, said alloy also having a minimum bend ductility of not over 20 T.

12. An alloy consisting essentially of about: 1 to 23% tin, 0.25 to 8% aluminum, up to 1% carbon, up to 0.5% oxygen, up to 0.4% nitrogen, 0.5 to 20% of at least one additional element selected from the group consisting of chromium and tungsten, balance titanium, characterized in having an ultimate strength substantially in excess of that of the corresponding base alloy without such addition, said alloy also having a minimum bend ductility of not over 20 T.

20 13. An alloy consisting essentially of about: 1 to 23% tin, 0.25 to 8% aluminum, up to 1% carbon, up to 0.5% oxygen, up to 0.4% nitrogen, 0.5 to 10% manganese, balance titanium, characterized in having an ultimate strength substantially in excess of the corresponding base alloy without such manganese addition, said alloy also having a minimum bend ductility of not over 20 T.

14. An alloy consisting essentially of about: 1 to 23% tin, 0.25 to 8% aluminum, up to 1% carbon, up to 0.5% oxygen, up to 0.4% nitrogen, 0.5 to 7% iron, balance titanium, characterized in having an ultimate strength substantially in excess of the corresponding base alloy without such iron addition, said alloy also having a minimum bend ductility of not over 20 T.

References Cited in the file of this patent

UNITED STATES PATENTS

2,669,513 Jaffee Feb. 16, 1954